

## UNITED STATES PATENT OFFICE

2,481,457

## GALVANIZING FLUX COMPOSITIONS AND PROCESSES

Charles A. Vana, Brecksville, Ohio, assignor to  
E. I. du Pont de Nemours & Company, Wil-  
mington, Del., a corporation of Delaware

No Drawing. Application February 3, 1945,  
Serial No. 576,162

6 Claims. (Cl. 148—23)

1

This invention relates to galvanizing fluxes and processes and more particularly to novel foaming fluxes having excellent fluidity and comprising a chloride, selected from the group consisting of ammonium chloride and zinc ammonium chloride, and an condensation product of formaldehyde corresponding to the formula



in which R and R' represent hydrogen, alkyl, amino, dimethyloacetyl, alpha-dimethylol-propionyl, or methyol groups, and is further particularly directed to galvanizing processes employing such fluxes.

In galvanizing practice it is customary to add a small amount of an organic material to the ammonium chloride or zinc ammonium chloride flux to produce a frothy layer on the surface of the molten metal in the galvanizing pot. A flux which in use forms such a frothy layer is known as a foaming flux. Organic materials commonly used to cause foaming are bran, glycerol, tallow, or sawdust. Inclusion of a foaming agent in a flux is ordinarily considered desirable because it retards decomposition of the flux, preheats incoming articles, and reduces spattering of molten metal.

Unfortunately, the foaming agents hitherto widely used have the disadvantage that after a period of use they thicken the flux and cause it to become viscous. This loss in fluidity is objectionable for a number of reasons. It retards the rate of wetting of the incoming work by the flux, which often results in failure to obtain complete coverage of the work and leads to imperfect galvanizing. It increases the rate at which flux is carried out on the finished work and complicates subsequent cleaning. It makes proper handling of the flux much more difficult. These and other objections to a viscous flux have caused some galvanizers in certain situations to prefer a non-foaming flux, despite the known advantages of foaming fluxes.

According to the present invention it has been found that by adding certain condensation products to ammonium chloride or zinc ammonium chloride there are produced galvanizing fluxes which are of the foaming type but which remain

2

remarkably fluid during use. The condensation products effective to produce this result are condensation products of formaldehyde corresponding to the formula



in which R and R' represent hydrogen, alkyl, amino, dimethyloacetyl, alpha-dimethylol-propionyl, or methyol groups. A further aspect of the invention consists of galvanizing processes employing such fluxes. The processes enjoy the advantages attending the use of a foaming flux but are not subject to the disadvantages heretofore ordinarily encountered. Moreover, by the use of a prepared flux composition of this invention the necessity for the galvanizer to determine the quantity of foamer to use is avoided.

To make a flux of this invention there is added to a major proportion of ammonium chloride or zinc ammonium chloride a minor proportion of a condensation product as a foamer. If too large a proportion of the foaming agent is used the flux will foam excessively and be difficult to use, while if the proportion is too small the advantages of the invention will not be fully realized. It has been found that the foaming agents herein described are extremely effective and it is preferred to employ about from 0.1 to 1.0 per cent by weight based on the ammonium chloride or zinc ammonium chloride.

The foamer may be added to the molten ammonium chloride or zinc ammonium chloride fluxing agent on the molten metal in the galvanizing pot. However, this involves the problem of distribution; that is, time and attention is required to insure a uniform distribution of the foamer throughout the fluxing agent. It is therefore preferred to incorporate the foamer in the fluxing agent prior to adding the flux to the galvanizing pot. This may be done by adding the foamer to the granular ammonium chloride or zinc ammonium chloride with mechanical agitation as, for instance, in a tumble mill. The products so produced are fluxes of maximum economy which can be used in the galvanizing plant with assurance of uniformity and without the close supervision attending the proportioning of the ingredients at the point of use.

The compounds employed as foamers in the fluxing compositions of this invention are either available commercially, for instance, pentaerythritol, or may easily be prepared by the condensation of formaldehyde with a suitable agent according to practices with which the art is already familiar.

In the following table are shown several examples of compounds which have been found to be effective as foamers in the fluxes of this invention, together with their structural formulae, their method of preparation, and the concentration of the agent, by weight, required in a zinc ammonium chloride flux to give a froth on a galvanizing bath during use equivalent to the froth produced by 0.75% glycerol, a foamer heretofore commonly used.

group and R represents a methylol group. In the case of 1-1, 3-3 tetramethylol 2-propanone, R' represents hydrogen and R represents an alkyl group.

The practice of this invention will be better understood by reference to the following illustrative example:

*Example*

10 Into the flux compartment of a job galvanizing pot, on the surface of the molten zinc, there was placed a quantity of a flux of this invention sufficient to produce a frothy layer about 15 inches deep. The flux used consisted of zinc ammonium chloride containing 0.37% of its weight of 15 pentaerythritol. Initially the molten flux layer had a viscosity of about 40 centipoises.

| Compound                                | Per Cent Conc. | Formula                                                                                                                                                                                                                   | Condensation Product of HCHO with: |
|-----------------------------------------|----------------|---------------------------------------------------------------------------------------------------------------------------------------------------------------------------------------------------------------------------|------------------------------------|
| Pentaerythritol.....                    | 0.37           | $  \begin{array}{c}  \text{CH}_2\text{OH} \\    \\  \text{HOCH}_2-\text{C}-\text{CH}_2\text{OH} \\    \\  \text{CH}_2\text{OH}  \end{array}  $                                                                            | Acetaldehyde.                      |
| Ethyl Trimethylol Methane.....          | 0.55           | $  \begin{array}{c}  \text{CH}_2\text{OH} \\    \\  \text{C}_2\text{H}_5-\text{C}-\text{CH}_2\text{OH} \\    \\  \text{CH}_2\text{OH}  \end{array}  $                                                                     | Butyraldehyde.                     |
| Methyl Trimethylol Methane.....         | 0.66           | $  \begin{array}{c}  \text{CH}_2\text{OH} \\    \\  \text{CH}_3\text{C}-\text{CH}_2\text{OH} \\    \\  \text{CH}_2\text{OH}  \end{array}  $                                                                               | Propionaldehyde.                   |
| Trimethylol Amino Methane.....          | 0.44           | $  \begin{array}{c}  \text{CH}_2\text{OH} \\    \\  \text{HOCH}_2-\text{C}-\text{NH}_2 \\    \\  \text{CH}_2\text{OH}  \end{array}  $                                                                                     | Nitromethane.                      |
| 2-Amino-2-Methyl 1,3 Propanediol.....   | 0.76           | $  \begin{array}{c}  \text{CH}_3 \\    \\  \text{HOCH}_2-\text{C}-\text{CH}_2\text{OH} \\    \\  \text{NH}_2  \end{array}  $                                                                                              | Nitroethane.                       |
| 1-1,3-3 Tetramethylol 2-propanone.....  | 0.48           | $  \begin{array}{c}  \text{CH}_2\text{OH} \\    \\  \text{HOCH}_2-\text{C}-\text{C}-\text{H} \\    \quad   \\  \text{H} \quad \text{O} \\    \\  \text{HOCH}_2-\text{C}-\text{CH}_2\text{OH}  \end{array}  $              | Acetone.                           |
| 2-Amino-2-Ethyl 1,3 propanediol.....    | 0.67           | $  \begin{array}{c}  \text{C}_2\text{H}_5 \\    \\  \text{HOCH}_2-\text{C}-\text{CH}_2\text{OH} \\    \\  \text{NH}_2  \end{array}  $                                                                                     | Nitroethane.                       |
| 1-1,3-3-Tetramethylol 2-butanone.....   | 0.48           | $  \begin{array}{c}  \text{CH}_2\text{OH} \\    \\  \text{H}_3\text{C}-\text{C}-\text{C}-\text{H} \\    \quad   \\  \text{HOCH}_2 \quad \text{O} \\    \\  \text{HOCH}_2-\text{CH}_2\text{OH}  \end{array}  $             | Methyl ethyl ketone.               |
| 2-2,4-4-Tetra-Methylol 3-Pentanone..... | 0.55           | $  \begin{array}{c}  \text{CH}_2\text{OH} \\    \\  \text{H}_3\text{C}-\text{C}-\text{C}-\text{C}-\text{CH}_3 \\    \quad   \\  \text{HOCH}_2 \quad \text{O} \\    \\  \text{HOCH}_2-\text{CH}_2\text{OH}  \end{array}  $ | Diethyl ketone.                    |
| 1-1,3-3 Tetramethylol 2-heptanone.....  | 0.70           | $  \begin{array}{c}  \text{CH}_2\text{OH} \\    \\  \text{H}-\text{C}-\text{C}-\text{C}-(\text{CH}_3)_3\text{CH}_3 \\    \quad   \\  \text{HOCH}_2 \quad \text{O} \\    \\  \text{CH}_2\text{OH}  \end{array}  $          | Methyl amyl ketone.                |

The foregoing compounds are all condensation products of formaldehyde and correspond to the formula



in which R and R' represent hydrogen, alkyl, amino, dimethylolacetyl, alpha-dimethylol-propionyl, or methylol groups. In the case of pentaerythritol, for instance, R and R' both represent methylol groups. In the case of ethyl trimethylol methane, R' represents an aliphatic

65 The galvanizing pot and flux bath were then used for galvanizing a quantity of iron pipe, the pipe being introduced into the molten zinc by passing through the frothing flux, then being passed beneath a dam holding back the flux, and being removed from the pot without again passing through the flux. During the operation additional flux was added as required to maintain the flux layer at its original depth. At the end of 70 eight hours of such operation the viscosity of the flux had risen to 200 centipoises but the flux was still sufficiently fluid to be effective, that is, it was 75 still a "live" flux.

For comparison, a similar operation was conducted in the same equipment under the same conditions and on the same type of work but using a zinc ammonium chloride flux containing 0.75% of glycerin as a foaming agent. Although this flux had about the same initial viscosity, viz. 43 cps., it was found that more frequent additions of flux during use were required to maintain the desired foam blanket, and after six hours the viscosity had risen to 240 cps. and the flux was considered "dead." During the six hour period of use the quantity of flux added to this bath was 15% greater than that added in the case of the pentaerythritol-containing flux during the corresponding period.

The work produced using the pentaerythritol-containing flux was uniformly well galvanized, being remarkably free of flux spots.

While in the foregoing description of this invention there have been shown certain particular compositions and processes, it will be understood that without departing from the spirit of the invention one skilled in the art may employ numerous compositions and processes.

I claim:

1. A foaming-type galvanizing flux consisting essentially of zinc ammonium chloride and pentaerythritol, the proportion of pentaerythritol being about from 0.1 to 1.0% by weight of the zinc ammonium chloride.

2. In a galvanizing process, the step comprising subjecting the work to be galvanized to contact with a flux consisting essentially of zinc ammonium chloride and pentaerythritol, the proportion of pentaerythritol being about from 0.1 to 1.0% by weight of the zinc ammonium chloride.

3. A foaming-type galvanizing flux consisting essentially of a fluxing agent selected from the group consisting of ammonium chloride and zinc ammonium chloride and about from 0.1 to 1.0% by weight based on the weight of fluxing agent, of a composition selected from the group consisting of pentaerythritol, ethyl trimethylol methane, methyl trimethylol methane, trimethylol amino methane, 2-amino-2-methyl 1,3 propanediol, 1-1,3-3 tetramethylol 2-propanone, 2-amino-2-ethyl 1,3 propanediol, 1-1,3-3-tetramethylol 2-butane, 2-2,4-4 tetramethylol 3-pentanone, and 1-1,3-3 tetramethylol 2-heptanone.

4. A foaming-type galvanizing flux consisting essentially of zinc ammonium chloride and about from 0.1 to 1.0% by weight based on the weight of zinc ammonium chloride, of a composition selected from the group consisting of pentaerythritol, ethyl trimethylol methane, methyl trimethylol methane, trimethylol amino methane, 2-amino-2-methyl 1,3 propanediol, 1-1,3-3 tetramethylol 2-propanone, 2-amino-2-ethyl 1,3 propanediol, 1-1,3-3 - tetramethylol 2 - butanone, 2-2,4-4 tetramethylol 3-pentanone, and 1-1,3-3 tetramethylol 2-heptanone.

5. In a galvanizing process, the step comprising subjecting the work to be galvanized to contact with a flux consisting essentially of a fluxing agent selected from the group consisting of ammonium chloride and zinc ammonium chloride and about 0.1 to 0.0% by weight based on the weight of fluxing agent, of a composition selected from the group consisting of pentaerythritol, ethyl trimethylol methane, methyl trimethylol methane, trimethylol amino methane, 2-amino-2-methyl 1,3 propanediol, 1-1,3-3 tetramethylol 2-propanone, 2-amino-2-ethyl 1,3 propanediol, 1-1,3-3-tetramethylol 2-butane, 2-2,4-4 tetramethylol 3-pentanone, and 1-1,3-3 tetramethylol 2-heptanone.

6. In a galvanizing process, the step comprising subjecting the work to be galvanized to contact with a flux consisting essentially of zinc ammonium chloride and about from 0.1 to 1.0% by weight based on the weight of zinc ammonium chloride, of a composition selected from the group consisting of pentaerythritol, ethyl trimethylol methane, methyl trimethylol methane, trimethylol amino methane, 2-amino-2-methyl 1,3 propanediol, 1-1,3-3 tetramethylol 2-propanone, 2-amino-2-ethyl 1,3 propanediol, 1-1,3-3-tetramethylol 2-butane, 2-2,4-4 tetramethylol 3-pentanone, and 1-1,3-3 tetramethylol 2-heptanone.

CHARLES A. VANA.

#### REFERENCES CITED

45 The following references are of record in the file of this patent:

#### UNITED STATES PATENTS

| Number       | Name   | Date          |
|--------------|--------|---------------|
| 50 2,311,669 | Kepfer | Feb. 23, 1943 |

Certificate of Correction

September 6, 1949

Patent No. 2,481,457

CHARLES A. VANA

It is hereby certified that errors appear in the printed specification of the above numbered patent requiring correction as follows:

Columns 3 and 4, in the table, third column thereof, opposite "Methyl Trimethylol Methane" for that portion of the formula reading



column 6, line 18, for "0.0%" read 1.0%;  
and that the said Letters Patent should be read with these corrections therein that  
the same may conform to the record of the case in the Patent Office.

Signed and sealed this 31st day of January, A. D. 1950.

[SNAL]

THOMAS F. MURPHY,  
*Assistant Commissioner of Patents.*